

## 1

2,961,408

## POWER TRANSMISSION MINERAL OIL BASE FLUIDS

Theodore W. Havelly, Alton, Stanley R. Sprague, East Alton, and Lawrence C. Westcott, Edwardsville, Ill., assignors to Shell Oil Company, New York, N.Y., a corporation of Delaware

No Drawing. Filed June 14, 1957, Ser. No. 665,660

13 Claims. (Cl. 252—75)

This invention pertains to improved functional fluids having good lubricating properties. More particularly this invention relates to mineral oil compositions for use in an apparatus by means of which mechanical forces are transmitted or absorbed such as in automotive and truck transmissions, hydraulic brakes, clutches, and various other mechanical equipment.

The smooth functioning of various power transmitting mechanisms particularly the more complicated automotive transmissions, fluid cooled brake mechanisms, oil lubricated wet clutches, planetary gears and hydraulic control mechanisms depends on adequate cooling and lubrication of the equipment. Rigorous requirements have been set up to quality fluids for this service which includes wide temperature stability at both high and low temperatures and a low pour point to insure proper pumpability and fluidity at low temperatures. The fluids must not have a detrimental effect on parts with which they come in contact such as metal surfaces e.g., copper and solid non-metallic surfaces such as organic resins and the like. They must possess desired frictional properties and, in some cases extreme pressure characteristics, to afford proper lubrication of gears, clutch plates and other parts of the mechanism in which they are used, such as automotive and truck equipment. Also, the fluids must not cause chattering, squawking, squealing or produce other noises caused by the frictional vibrations and/or stick-slip phenomenon of clutch plates or other parts of such mechanisms.

The prior art discloses various functional or power transmission fluids of the mineral oil or synthetic type (organic esters and polyethers) containing as the improving agents, various organic phosphates, fatty acids and their esters, halogenated compounds, polymers such as polyacrylates and the like. Compositions of this type are objectionable because of their inability to eliminate chattering and noises caused by frictional vibrations and/or stick-slip phenomenon of clutch plates and the like, particularly in equipment which is subjected to high speeds and temperatures.

It has now been discovered that an excellent functional or power transmission fluid is provided, which satisfactorily meets the above requirements, which comprises a highly refined mineral oil base containing an additive combination, in critical amounts, of from about 0.05% to about 2%, preferably from about 0.1% to about 1% each of (1) a saturated aliphatic monocarboxylic acid having at least 18 carbon atoms in the molecule and (2) a product of neutralization between an aliphatic amine having at least 8 carbon atoms with a mono- or di-aliphatic acid pyrophosphate having at least 8 carbon atoms.

The long-chain aliphatic monocarboxylic acids include the saturated fatty acids of the  $C_{18}$  to  $C_{30}$  range such as stearic, arachidic, behenic, cerotic, montanic acids and mixtures thereof. Preferred are of saturated fatty acids having 18 to 26 carbon atoms such as stearic acid, behenic acid and cerotic acid and their mixtures.

The second essential additive is a product of neutral-

## 2

ization between an aliphatic amine having at least 8 carbon atoms and a mono- or dialiphatic acid pyrophosphate the aliphatic group containing at least 8 carbon atoms. The aliphatic amines suitable for reaction with the aliphatic acid pyrophosphates are the primary and secondary saturated or unsaturated aliphatic amines having from 8 to 18 carbon atoms or mixtures of such amines. Typical of such amine reactants are octylamine, dodecylamine, tetradecylamine, hexadecylamine, octadecylamine, octadecenylamine, octadecadienylamine, di-octylamine, diodoctylamine, dioctadecylamine, dioctadecadienylamine and amines derived from fatty oils or fats such as cottonseed oil, soybean oil, coconut oil; lard, tallow, and the like, such as soyamine, cocoamine, tallowamine and mixtures thereof. Amines of this type are marketed by Armour and Co. under the trade name "Armeen" and include "Armeen 12 and 12 D" (dodecylamine), "Armeen 14 and 14 D" (tetradecylamine) "Armeen 16 and 16 D" (hexadecylamine) "Armeen 18 and 18 D" (octadecylamine), "Armeen TD" (mixture of tetradecyl, hexadecyl and octadecylamines), "Armeen S and SD" (mixtures of hexadecyl, octadecyl, octadecenyl and octadecadienyl amines). Preferred are the unsaturated amines such as octadecadienylamine or "Armeen S" and "Armeen SD." Polyamines are also included as reactants with the pyrophosphates. Polyamines which are preferred are the N-alkyl alkene diamines which are prepared by the method described in U.S. 2,736,658 and are marked by Armour and Co. under the trade name "Duomeens" such as "Duomeen C," "Duomeen S" and "Duomeen T," which are  $C_{12-18}$  alkyl trimethylene diamines, derived from coconut, soybean and tallow respectively. Polyamines of this type are also available from General Mills under the trade name "Diams."

35 The mono or dialiphatic acid pyrophosphates include mono- and dioctyl pyrophosphate, mono- and didodecyl pyrophosphate, mono- and ditetradecyl pyrophosphate, mono- and di-hexadecyl pyrophosphate, mono- and di-octadecyl pyrophosphate, of which preferred are mono-octyl pyrophosphate dioctyl pyrophosphate, monododecyl pyrophosphate, didodecyl pyrophosphate, mono-octadecyl pyrophosphate, dioctadecyl pyrophosphate and mixtures thereof.

The reaction between the amine and the pyrophosphate is exothermic and should be controlled so as to prevent decomposition. Generally the temperature of the reaction should be between 50 and 100° C. and preferably below 80° C. The mol ratio of the reactants should be within the ratio of 1 to 5 moles of the amine per mol of pyrophosphate compound, and preferably the reactants and reaction should be carried out under such conditions that the end product contains no free acid but can contain some free amine.

The amine-acid pyrophosphate reaction products in the molar proportions indicated in Table I were made as follows:

TABLE I

| Example | Amine                  | Acid pyrophosphate    | Molar ratio of amine to pyrophosphate | Temperature, °C. |
|---------|------------------------|-----------------------|---------------------------------------|------------------|
| I       | Armeen SD <sup>1</sup> | Dioctylpyrophosphate  | 2/1                                   | 70               |
| II      | do                     | do                    | 5/1                                   | 70               |
| III     | do                     | do                    | 2.5/1                                 | 70               |
| IV      | Octadecylamine         | Lauryl pyrophosphate  | 5/1                                   | 80               |
| V       | Dodecylamine           | Dodecyl pyrophosphate | 5/1                                   | 80               |
| VI      | Duomeen T <sup>2</sup> | Dioctylpyrophosphate  | 4/1                                   | 70               |

<sup>1</sup> Armeen SD = mixture of 10% hexadecylamine, 10% octadecylamine, 35% octadecenylamine and 45% octadecadienylamine.

<sup>2</sup> Duomeen T =  $C_{12-18}$  trimethylene diamine derived from tallow.

Functional fluids of the above type are noise-free and their static coefficient of friction is low. For certain applications the static coefficient of friction of such noise-free functional fluids should be high, as in fluids used in parking-brakes or the like, where it is desired that the frictional level be high enough (at least  $0.125\mu$ ) so that the force generates a frictional torque level sufficient to overcome the gravitational pull on a 30° incline. A class of additives which when added, in amounts of from about 0.1% to about 10%, preferably from about 0.5% to 5% by weight, to functional fluids of this invention, increase their static coefficient of friction to at least  $0.125\mu$  are oil-soluble alkali metal or alkaline earth metal organic sulfonates. Materials for making oil-soluble sulfonates include various petroleum fractions such as mineral lubricating oil fractions, alkyl-substituted aromatic compounds such as alkylated benzene or naphthalene and alkyl substituted polar-containing aromatic compounds such as alkylated phenol, naphthol, aniline, etc. Specific sulfonates which are particularly suitable for increasing the static coefficient of friction of functional fluids of this invention oil-soluble sodium, potassium, calcium and barium petroleum sulfonate, tetra-tertiary butylnaphthalene sulfonate, dinonyl naphthalene sulfonate, diwaxnaphthalene sulfonate, diwaxbenzene sulfonate, stearylbenzene sulfonate, tertiary-octylphenol sulfonate, waxphenol sulfonate and mixtures thereof. Preferred are the oil-soluble sodium, calcium and/or barium petroleum sulfonate and dinonylnaphthalene sulfonate.

In addition to the two essential additives present in compositions of this invention, as well as the frictional additive (sulfonate), it is preferred to incorporate into such compositions a small amount (0.1-5%) of specific anti-oxidants from groups (a) an oil-soluble organic thiophosphate salt of the metals of group II of the periodic table having an atomic number of from 12 to 56 or (b) a mixture in about equal proportions of an alkyl phenol and an arylamine. The anti-oxidant of group (a) include the group II metal salts of alkyl, aryl, alkaryl, or cycloalkyl mono- and di-acid thio or dithio-phosphoric acids such as calcium, barium or zinc alkyl, cyclo alkyl or aryl mono and dithiophosphates. Preferred compounds are calcium, barium and zinc methylphenyl dithiophosphate, dimethyl cyclohexyl dithiophosphate, dihexyl dithiophosphate, lauryl benzyl dithiophosphate and mixtures thereof. Compounds of this type are available commercially under the trade names of Lubri-Zol 66, 304, 360 or 1060 (Lubri-Zol Corp.); Aerolube 70 (American Cyanamid Co.) and Stan-Add 71 (Standard Oil Co. of Indiana). A particularly preferred class of such compounds includes the Zn and Ba salts of dimethylcyclohexyl dithiophosphate, Ba salt of  $P_2S_5$ -polybutene reaction products and/or  $P_2S_5$ -terpene (pinene) reaction products. Such products are commercially available from Lubri-Zol Corporation, Standard Oil Company of Indiana and Monsanto Chemical Company, respectively, under the above indicated trade names.

The anti-oxidant mixture of group (b) include alkyl phenols, e.g., di and tri alkylphenols, for instance 2,4-, 2,3-, 3,4-, 2,6- and 3,5-diamyl phenol, 2,4-dimethyl-6-tertbutyl phenol, 2,6-ditertbutyl-4-methyl phenol; and arylamines such as phenyl- $\alpha$ -naphthylamine, or phenyl- $\beta$ -naphthylamine.

Also optional additives can be used in compositions of this invention such as anti-foaming agent e.g., silicone polymers (DC 200 fluids) ranging in viscosity in centistokes from 100 to 1000 at 25° C. or Silicone Type A fluid made by Dow-Corning Co. and described in U.S. Patents 2,563,588 and 2,662,055. These optional agents when used in compositions of this invention are employed in amounts of from 0.0001% to 10% and preferably between 0.1% and 5%.

The base oil is a hydrocarbon oil preferably of wide viscosity range and having a high viscosity index and a low pour point. These oils can range in viscosity from 40

SUS at 100° F. to 150 SUS at 210° F., and include mineral spray oil, transformer oil as well as lubricating oils having SAE numbers of 10, 20, 30, etc. Oils of this type have the following properties:

|    |                            |      |
|----|----------------------------|------|
| 5  | SAE 10 mineral oil         |      |
|    | Viscosity, SUS, at 100° F. | 175  |
|    | Viscosity, SUS, at 210° F. | 45.2 |
|    | Viscosity index            | 106  |
| 10 | Flash, ° F.                | 395  |
|    | Fire, ° F.                 | 440  |
|    | Pour point, ° F.           | —35  |

Another suitable base oil is a refined, highly refined transformer oil (A) having the following properties:

|    |                            |           |
|----|----------------------------|-----------|
| 15 | Sp. gr., ° API             | 30.9      |
|    | Color                      | 30        |
|    | Viscosity, SUS, at 100° F. | 56.9      |
|    | Flash, COC, ° F.           | 290       |
| 20 | Fire, COC, ° F.            | 320       |
|    | Pour point, ° F.           | Below —70 |

Still another suitable base oil is a refined mineral oil (B) having the following properties:

|    |                            |      |
|----|----------------------------|------|
| 25 | Sp. Gr., ° API             | 31.2 |
|    | Color, ASTM                | —1   |
|    | Pour point                 | —30  |
|    | Flash, ° F.                | 270  |
|    | Fire, ° F.                 | 295  |
| 30 | Viscosity, SUS, at 100° F. | 48   |
|    | Viscosity index            | 33   |

The following compositions are illustrative of the present invention.

#### Composition A

|    |                                                |            |     |
|----|------------------------------------------------|------------|-----|
| 35 | Stearic acid                                   | percent wt | 0.2 |
|    | Example I additive                             | do         | 0.2 |
|    | Calcium petroleum sulfonate                    | do         | 5   |
|    | Zinc dimethyl cyclohexyl dithiophosphate       | do         | 0.5 |
| 40 | Dimethyl silicone polymer (1000 cs. at 25° C.) | p.p.m.     | 5   |
|    | Mineral oil (B)                                | Balance    |     |

#### Composition B

|    |                                               |            |     |
|----|-----------------------------------------------|------------|-----|
| 45 | Stearic acid                                  | percent wt | 0.2 |
|    | Example I additive                            | do         | 0.2 |
|    | 2,6 ditertbutyl-4-methylphenol                | do         | 0.2 |
|    | Phenyl- $\alpha$ -naphthylamine               | do         | 0.1 |
| 50 | Dimethyl silicone polymer (500 cs. at 25° C.) | p.p.m.     | 5   |
|    | Transformer oil (A)                           | Balance    |     |

#### Composition C

|    |                                               |            |     |
|----|-----------------------------------------------|------------|-----|
| 55 | Stearic acid                                  | percent wt | 0.2 |
|    | Example II additive                           | do         | 0.2 |
|    | Dimethyl silicone polymer (500 cs. at 25° C.) | p.p.m.     | 5   |
|    | Transformer oil (A)                           | Balance    |     |

#### Composition D

|    |                     |            |     |
|----|---------------------|------------|-----|
| 60 | Cerotic acid        | percent wt | 0.3 |
|    | Example VI additive | do         | 0.2 |
|    | Transformer oil (A) | Balance    |     |

Compositions of this invention eliminate noise, frictional vibrations and stick-slip sliding in various equipment such as liquid cooled hydraulic brake systems in which the friction members were made of steel and resilient, or semi-metallic, or full sintered metallic friction materials. Evaluation was done in actual automobile tests wherein the noise created after accelerating and suddenly stopping the vehicle was rated, 10 being excellent, no noise or stick-slip and zero (0) being poor, severe noise and stick-slip.

With compositions A, B, C, and D the ratings were between 8 and 10. Mineral oils (A) and (B), each containing 0.2% stearic acid, or 0.2% cerotic acid gave

ratings of 4 and 5 respectively, while the same oils each containing 0.2% stearic acid and 5% Lubri-Zol 66 gave ratings of 5. Transformer oil (A) or mineral oils (B) each containing 0.5% of n-octyl acid phosphate, dioctyl phosphate and triisoctyl phosphate gave ratings of 4, 1 and 1, respectively, while transformer oil (A) containing 0.4% lauryl acid phosphate gave a rating of 3 and transformer oil (A) containing 0.2% lauryl acid phosphate and 2.5% "Lubri-Zol 1060" gave a rating of 1.

The static coefficient of friction of Compositions B, C and D was about  $0.04\mu$  whereas the static coefficient of friction of Composition A containing 2.5% neutral calcium petroleum sulfonate increased the coefficient of friction to  $0.130\mu$ . The addition of 2.5% of neutral calcium dinonylnaphthalene sulfonate or barium dinonylnaphthalene sulfonate, or neutral calcium petroleum sulfonate to Composition C increased the static coefficient of friction of the compositions from  $0.04\mu$  to  $1.52\mu$ ,  $1.88\mu$  and  $1.42\mu$ , respectively. These values are far above the required minimum of  $0.125\mu$ . On the other hand, the addition of 2.5% of calcium naphthenate, or calcium  $C_{14-18}$  alkyl salicylate, or zinc dimethylcyclohexyl dithiophosphate or tricresyl phosphate to Composition C gave static coefficient of friction values of  $0.086\mu$ ,  $0.49\mu$ ,  $0.052\mu$  and  $0.091\mu$ , respectively. These values are below the required minimum of  $0.125\mu$ .

Thus the data shows the outstanding properties which compositions of this invention possess with respect to eliminating noise and stick-slip in brake systems. On the other hand, mineral oils containing a fatty acid, e.g., stearic or cerotic acids alone or in combination thiophosphates or mineral oils containing various acid phosphates alone or in combination with a metal thiophosphate gave poor results. Also the data shows that the static coefficient of friction of compositions of the present invention can be increased to a desired value by addition to such compositions certain oil-soluble sulfonates and that other metal salts e.g. naphthenates or salicylates or phosphate esters are not effective when used for this purpose in compositions of this invention.

We claim as our invention:

1. A noise-free power transmission fluid consisting essentially of a major amount of a refined mineral lubricating oil and from about 0.05% to about 2% each of an aliphatic monocarboxylic acid having from 18 to 26 carbon atoms in the molecule and a reaction product prepared by reacting from 1 to 5 moles of an aliphatic amine having from 8 to 18 carbon atoms with a mol of an aliphatic acid pyrophosphate having from 8 to 18 carbon atoms until the reaction is substantially completed, the reaction being carried out at a temperature below that at which substantial decomposition of the reaction product occurs.

2. A noise-free power transmission fluid consisting essentially of a major amount of a refined mineral lubricating oil and from about 0.05% to about 2% each of a saturated fatty acid having from 18 to 26 carbon atoms in the molecule and a reaction product prepared by reacting from 1 to 5 moles of a  $C_{8-18}$  aliphatic amine with a mol of an aliphatic acid pyrophosphate having from 8 to 18 carbon atoms until the reaction is substantially completed, the reaction being carried out at a temperature below that at which substantial decomposition of the reaction product occurs.

3. A noise-free power transmission fluid consisting essentially of a major amount of a refined mineral lubricating oil and from 0.05% to about 2% each of a saturated fatty acid having from 18 to 26 carbon atoms in the molecule and a reaction product prepared by reacting from 1 to 5 moles of a  $C_{8-18}$  alkyl amine with a mol of an alkyl acid pyrophosphate having from 8 to 18 carbon atoms until the reaction is substantially completed, the reaction being carried out at a temperature below that at which substantial decomposition of the reaction product occurs.

4. A noise-free power transmission fluid consisting es-

sentially of a major amount of a refined mineral lubricating oil and from about 0.05% to about 2% each of stearic acid and a reaction product of a  $C_{8-18}$  aliphatic amine with a mol of an alkyl pyrophosphate having from 8 to 18 carbon atoms until the reaction is substantially completed, the reaction being carried out at a temperature below that at which substantial decomposition of the reaction product occurs.

5. A noise-free power transmission fluid consisting essentially of a major amount of a refined mineral lubricating oil and from about 0.05% to about 2% each of stearic acid and a reaction product prepared by reacting from 1 to 5 moles of a  $C_{8-18}$  aliphatic amine with a mol of octyl pyrophosphate until the reaction is substantially completed, the reaction being carried out at a temperature below that at which substantial decomposition of the reaction product occurs.

6. A noise-free power transmission fluid consisting essentially of a major amount of a refined mineral lubricating oil and from about 0.05% to 2% each of stearic acid and a reaction product prepared by reacting from 1 to 5 moles of a  $C_{8-18}$  aliphatic amine with a mol of dioctyl pyrophosphate until the reaction is substantially completed, the reaction being carried out at a temperature below that at which substantial decomposition of the reaction product occurs.

7. A noise-free power transmission fluid consisting essentially of a major amount of a refined mineral lubricating oil and from about 0.05% to 2% each of cerotic acid and a reaction product prepared by reacting from 1 to 5 moles of a  $C_{8-18}$  aliphatic amine with a mol of an alkyl pyrophosphate having from 8 to 18 carbon atoms until the reaction is substantially completed, the reaction being carried out at a temperature below that at which substantial decomposition of the reaction product occurs.

8. The power transmission fluid of claim 1 containing from about 0.1% to about 10% of an oil-soluble metal organic sulfonate the metal portion of the salt being selected from the group consisting of alkali and alkaline earth metals.

9. The power transmission fluid of claim 4 containing from about 0.1% to 10% of oil-soluble calcium petroleum sulfonate and from about 0.1% to about 5% of oil-soluble zinc cycloalkyl dithiophosphate.

10. The power transmission fluid of claim 5 containing from about 0.1% to 10% of oil-soluble sodium petroleum sulfonate.

11. A noise-free power transmission fluid consisting essentially of about 0.2% stearic acid, about 0.2% of a reaction product prepared by reacting from 1 to 5 moles of  $C_{16-18}$  aliphatic amine with a mol of dioctyl pyrophosphate until the reaction is substantially completed, the reaction being carried out at a temperature below that at which substantial decomposition of the reaction product occurs, and about 0.1-0.5% of a mixture of an alkyl phenol and an aryl amine and the balance being a refined transformer mineral oil.

12. A noise-free power transmission fluid consisting essentially of about 0.2% stearic acid, about 0.2% of a reaction product prepared by reacting from 1 to 5 moles of  $C_{16-18}$  aliphatic amine with a mol of dioctyl pyrophosphate until the reaction is substantially completed, the reaction being carried out at a temperature below that at which substantial decomposition of the reaction product occurs, about 0.2% of 2,6 tertiary-4-methyl phenol, about 0.1% of phenyl- $\alpha$ -naphthylamine, and about 5 p.p.m. of dimethyl silicone polymer, the balance being a refined transformer mineral oil.

13. A noise-free power transmission fluid consisting essentially of about 0.2% stearic acid, about 0.2% reaction product prepared by reacting from 1 to 5 moles of  $C_{16-18}$  aliphatic amine with a mol of dioctyl pyrophosphate until the reaction is substantially completed, the reaction being carried out at a temperature below that at which substantial decomposition of the reaction product occurs, about

2.5-5% calcium petroleum sulfonate, about 0.5% zinc dimethylcyclohexyl dithiophosphate, and about 5 p.p.m. dimethyl silicone polymer and the balance being a refined transformer mineral oil.

**References Cited in the file of this patent**

**UNITED STATES PATENTS**

2,005,619    Graves    June 18, 1935

|           |                  |               |
|-----------|------------------|---------------|
| 2,080,299 | Benning          | May 11, 1937  |
| 2,447,483 | Baker            | Aug. 24, 1948 |
| 2,509,620 | Watson           | May 30, 1950  |
| 2,595,170 | Rudel            | Apr. 29, 1952 |
| 2,664,400 | Woodstock et al. | Dec. 29, 1953 |
| 2,686,760 | Watson           | Aug. 17, 1954 |
| 2,694,045 | Jones            | Nov. 9, 1954  |
| 2,830,956 | Wasson et al.    | Apr. 15, 1958 |
| 2,848,414 | Chenicek         | Aug. 19, 1958 |